

Sept. 24, 1929.

J. A. GANN

1,729,339

ALLOY OF MAGNESIUM

Filed Oct. 27, 1921



Mg + Cd

INVENTOR  
*John A. Gann*  
BY  
*Day, Oberlin & Day*  
ATTORNEYS

## UNITED STATES PATENT OFFICE

JOHN A. GANN, OF MIDLAND, MICHIGAN, ASSIGNOR TO THE DOW CHEMICAL COMPANY, OF MIDLAND, MICHIGAN, A CORPORATION OF MICHIGAN

## ALLOY OF MAGNESIUM

Application filed October 27, 1921. Serial No. 510,795.

The present improved alloy is one in which magnesium is the predominant element, the object being to develop an alloy that will possess the characteristic lightness which is obtained by the use of magnesium in excess of 80%, while such alloy will be characterized by high strength and toughness, as well as have a high melting point and high thermal conductivity.

10 The field of use in the mechanical arts to which an alloy possessing the lightness and physical characteristics enumerated above may be applied need not be described in detail for the purpose in hand, especially when it is added that the particular alloy herein-after described possesses the added quality of mechanical workability, i. e., it may be readily forged or shaped under pressure, rolled into sheets or drawn. Where hardness rather than softness may be considered desirable, as, for example, where the metal is to be used in pistons of internal combustion engines this characteristic may be improved by adding one or more other metals in varying quantities, as will be hereinafter explained, the present invention consisting of an alloy of magnesium and cadmium with or without the addition of such further metals, together with the steps involved in the making of such alloy 15 hereinafter fully described and particularly pointed out in the claims. The annexed drawing and following description, it will be understood, set forth but several of the various ways in which the invention may be carried out.

In said annexed drawing:-

The single figure there appearing is a diagrammatic representation of certain physical properties discovered in a binary magnesium-cadmium alloy of the class in hand. In such diagrammatic figure, the physical properties represented, it will be noted, are the impact-toughness, hardness and tensile strength, the hardness being determined by the Brinell method and scaled to correspond with the impact-toughness, the latter being determined by the single-blow method. While such impact-toughness drops rapidly up to the addition of 4 per cent of cadmium, it will be observed that from this point on the curve

becomes much less steep with the addition of more cadmium. The tensile strength, on the contrary, increases rapidly at first and then at a rate approximately inverse to the rate of decrease in impact-toughness. The 55 Brinell hardness increases slowly and at a practically constant rate throughout the range under consideration, which I place at between 5% and 10% of cadmium in order to secure a proper balance in respect to the 60 characteristics in question.

The resulting alloy, where between 5% and 10% of cadmium is thus utilized, the balance being magnesium, will have a specific gravity varying from approximately 1.8 to 65 1.9; tensile strength, from 19,000 to 20,500 per square inch; Brinell hardness, from 44 to 45; and single blow impact-toughness from 90 to 85.

Where the alloy is to be used for pistons in internal combustion engines, or under conditions involving similar strains and temperatures, I have found that the addition of a small proportion of aluminum or of aluminum and copper is advantageous in that 70 it imparts increased hardness in the resulting product. A satisfactory formula for such a ternary alloy in which aluminum is the third ingredient is as follows, viz:—magnesium 88%, cadmium 8% and aluminum 80 4%; for such a ternary alloy in which copper is the third ingredient the preferred formula is as follows, viz:—magnesium 94%, cadmium 4% and copper 2%; while for an alloy including both aluminum and copper 85 the following composition is recommended, viz:—magnesium 88%, cadmium 6%, aluminum 4% and copper 2%.

Even where the proportion of aluminum thus added is greater than that of the cadmium, as in the following formula, viz, magnesium 90%, aluminum 8%, copper 1% and cadmium 1%, the characteristics noted above as having been discovered in the simple binary alloy of magnesium and cadmium 90 will be retained to a perceptible degree. This may be attributed to the fact that cadmium forms a solid solution with magnesium throughout the whole series of possible combinations. In other words, there is no 95 100

eutectic present whatever the proportion of cadmium. A relatively high melting point is also obtained, as well as a high thermal conductivity, the latter being 0.304, where the 5 proportion of cadmium is 12%, or only a little less than the thermal conductivity of pure magnesium, and correspondingly nearer that of magnesium where the proportion of cadmium is less. So far as concerns impact- 10 toughness, as determined by the single blow method in the range beyond 5% of cadmium and up to 20%, the present binary alloy shows greater toughness than any binary magnesium alloy with another metal present in 15 corresponding amount.

To make my improved alloy a measured quantity of pure magnesium metal is first melted in a suitable pot along with a proper amount of flux that, while heavier than such 20 metal, will have proper surface tension to properly and effectively coat the metal. As an example of such a flux, approximately equal parts of anhydrous magnesium chloride and sodium chloride may be employed 25 and if the specific gravity of such flux proves inadequate to float the metal after it has been alloyed, a small amount of barium chloride may be added. A small amount of the molten magnesium metal is then taken up into 30 the ladle and all or a part of the cadmium, depending on the total percentage of the latter to be added to the batch, is first placed in such ladle and melted with the magnesium therein, thereby producing an alloy relatively 35 high in cadmium. The contents of the ladle are then gradually added to the main body of molten magnesium, with the result that the cadmium will diffuse throughout the mass and not drop into the body of flux on which 40 the latter floats and so be lost. As soon as the introduction of the cadmium alloy has been effected, the whole mass is then well puddled, and the operation may then be regarded as complete and the molten alloy cast either 45 into ingots or directly into the form of mechanical parts, such as pistons or the like, for which it is intended to be used.

Where aluminum, or aluminum and copper, or other metals are to be added to the 50 binary alloys in accordance with the illustrative formulas hereinbefore given, such additional metal or metals may be separately introduced in the same fashion as the cadmium, or they may be at once added along with the 55 cadmium in forming the preliminary alloy which is subsequently added to the main body of the molten magnesium metal, resulting in the production of an alloy in which magnesium is the predominant ingredient. Again, 60 in some cases it may be found more advantageous to add to the magnesium alloy in the ladle a magnesium alloy rich in the alloying metal, instead of such metal itself.

For convenience in defining the relative 65 proportions of the metals that enter into the

alloy, the magnesium may be referred to as present in predominant amount, meaning an amount on the order of 80 per cent or more of the total; while in referring to the presence of other constituents in substantial but 70 relatively small amounts, it will be understood that amounts are meant on the order of those specified in the formulas hereinbefore set forth, due regard being given to the fact that the total of such other ingredients will 75 decrease as the amount of the predominant constituent is increased.

Other modes of applying the principle of my invention may be employed instead of the one explained, change being made as regards 80 the steps herein disclosed or the ingredients employed in carrying out such steps, provided the steps or ingredients set forth in the following claims, or the equivalent of such steps or ingredients be employed.

I therefore particularly point out and distinctly claim as my invention:—

1. As a new product, an alloy containing from ninety to ninety-five per cent of magnesium and between ten and five per cent of 90 cadmium.

2. As a new product, an alloy containing magnesium, cadmium, aluminum and copper, wherein the magnesium largely predominates and the remaining constituents are present in 95 substantial but relatively small amounts.

3. As a new product, an alloy containing magnesium, cadmium, aluminum and copper, wherein the magnesium largely predominates and the remaining constituents are present 100 in substantial but relatively small amounts, the cadmium being the principal other ingredient.

4. As a new product, an alloy containing approximately the indicated percentages of 105 the following metals, viz:—magnesium eighty-eight per cent, cadmium eight per cent and aluminum four per cent.

5. The method of making a magnesium-cadmium alloy, which consists in first inter-fusing the desired amount of cadmium with a relatively small quantity of magnesium, and then adding the resulting alloy to the remaining quantity of magnesium in molten state.

6. The method of making a magnesium-cadmium alloy, wherein the magnesium largely predominates, which consists in first inter-fusing the desired amount of cadmium with a relatively small quantity of magnesium, whereby an alloy high in cadmium is produced, and then adding such resulting alloy to the remaining quantity of magnesium.

Signed by me this 24th day of October, 1921.

JOHN A. GANN.